

## UNITED STATES PATENT OFFICE

2,304,089

PROCESS OF PRODUCING ARTIFICIAL  
FIBROUS MATERIAL

Georg Heberlein, Wattwil, Switzerland

No Drawing. Application April 4, 1941, Serial  
No. 386,837. In Germany April 9, 1940

3 Claims. (Cl. 57—157)

This invention relates to the improvement of artificial fibers, and is especially useful in connection with the treatment of artificial silk according to the U. S. Patents 2,019,185 or 2,019,183.

Following the first-called specification a wool-like artificial silk results by supertwisting a normal twisted or not twisted artificial silk yarn, setting the twist therein for instance by moistening and drying it on bobbins at a high temperature and afterwards untwisting the yarn giving to it preferably a light twist in the opposite direction.

Following the second specification a further improvement consists therein that the yarn after untwisting it, is exposed to a wet heated atmosphere in a loose i. e. untensioned state.

One advantage of my invention in comparison with the before mentioned processes consists therein that it will be possible by the new process to obtain durable wool effects. Under durable wool effects I understand permanent effects especially wool effects which resist the mechanical influences during weaving, knitting and further finishing as well as to laundering of the goods, made out of such yarns.

A further advantage of the material manufactured according to my process is that it does not change its character during the wearing of clothes or the use of textiles made therefrom.

As another advantage of my process I mention that it renders commercially dyed goods more fast to washing.

Another advantage consists therein that yarns produced according to my process and clothes or knitted goods manufactured from these yarns show a reduced tendency to shrink on laundering.

According to my invention artificial silk preferably produced as described in the above-mentioned patent specifications is treated with formaldehyde or formaldehyde yielding substances and in the presence of acid reacting catalysts at temperatures of preferably 90—160° C.

The process may be applied to any sort of artificial fibers capable of reacting with formaldehyde, such as artificial fibers of regenerated cellulose. It is useful to treat with formaldehyde following the processes described in the Patents 2,019,185 or 2,019,183, but it is also possible to treat with formaldehyde at an earlier stage or to combine the formaldehyde treatment with the steaming or drying step. If coloured yarns are desired it is suitable to dye with naphtole- or vat dyestuffs, for instance before supertwisting and before the formaldehyde treatment is applied.

If direct dyestuffs are used it will be advantageous to dye before supertwisting, as otherwise it is often difficult to obtain even shades. As to the election of dyestuffs, such dyestuffs may be used which do not or do only slightly alter their colour shade by a treatment with formaldehyde. In general these are the same dyestuffs recommended by the dyestuff factories for finishing crease-resistant goods.

10 It will also be possible to combine the formaldehyde treatment with a finish to render the yarns at the same time water repellent, for instance with stearyl- or montanyl-isocyanates or octadecyloxymethyl-pyridium chloride. Generally the wool effect is developed on exposing the formerly supertwisted steamed and untwisted yarn loosely to the air; steaming will accelerate the curling of the yarn. In the case that the yarn is to be further treated or used under tension for instance on bobbins to be woven in a pile fabric then the wool effect may be developed advantageously by steaming after the weaving and cutting off. It may even be of advantage in such a case to treat with the formaldehyde after weaving. Pile fabrics manufactured according to my process are characterised by a full hand, great tightness and uniform appearance.

15 The formaldehyde treatment corresponds generally to the treatment described in the specification of the copending Frauenfelder continuing application No. 357,119 filed on September 17, 1940, and examples are given below.

20 As suitable catalysts there are employed strong acids, especially mineral acids or their ammonium salts, such for example as ammonium chloride. Other suitable catalysts are metal salts of such acids such for example as aluminium salts. Specially as catalysts I mention the following mineral acids, nitric acid, phosphoric acid and their at elevated temperatures acid reacting salts; soluble aluminium salts such as aluminium chloride, aluminium sulphate, aluminium thiocyanate or the like. In addition there may also be employed zinc chloride and ammonium thiocyanate. In practice I have used a highly dissociated acid or a substance yielding such an acid at elevated temperatures and preferably a suitable salt of a highly dissociating acid such for example as ammonium chloride and zinc chloride, as such salts seem to have a buffer action giving better control of the reaction between the formaldehyde and cellulose so as to assist in avoiding or minimizing damage to the fabric. By the term "highly dissociated acid" as used herein 25 I wish to include not only those acids which are

25

30

35

40

45

50

55

strictly classified as highly dissociated, but also those which are moderately dissociated i. e. those having a dissociation constant above  $3 \times 10^{-4}$ .

The formaldehyde is preferably applied to the yarn by impregnating it with a solution of technical formaldehyde. To this impregnating bath the catalysts may be added. After squeezing out and drying the goods are submitted to heating in dry state.

Depending on the material to be worked, the impregnation can be carried out in a cold or hot bath. The duration of the impregnation period also is varied according to the kinds of goods employed. The goods may be subjected to 60-90° C. for drying and afterdrying the temperature is elevated at about 90-160° C., but with temperature above about 130° C. great care must be exercised. The duration and temperature of the heating is governed to some extent by the catalyst and kind of material employed. At a low temperature, for instance 100° C. obviously longer treating may be employed, while at higher temperatures a shorter period of heating is ordinarily employed. The treatment with formaldehyde or its compounds with the catalysts herein described and at the temperature stated for the period of time given herein causes a reaction between the formaldehyde and cellulose and a compound of cellulose and formaldehyde is formed. The content of chemically bound formaldehyde in the cellulose may be analytically tested and must generally surpass 0.15% to show the desired effects.

Although formaldehyde treatments of cellulose are known per se, the effects which I obtain have never been described and the result of submitting yarns such as those treated according Patents 2,019,185 or 2,019,183 to a formaldehyde treatment could not be foreseen. It was however known that calander and gaufrage effects could be fixed by a formaldehyde treatment under certain condition, but if one would try to fix such effects following the methods preferred and described in the examples thereafter, the result would be zero.

The following are examples of the process and it is to be understood that the examples are purely illustrative and that the invention is not restricted thereto.

*Example 1.*—Viscose artificial silk yarn of a size of 450 denier with a twist of 100 per meter is supertwisted to 1200 twists per meter. Thereupon the supertwisted yarn which has been placed on bobbins is steamed at 2 atmospheres pressure for half an hour. After drying the yarn is untwisted past the zero point and brought to 50 twists per meter in the opposite direction. The resulting yarn is formed into hanks and is wool-like. Afterwards the wool-like or curled hanks are impregnated with a solution of 200 cc. formaldehyde 40% and 40 cc. solution of aluminium thiocyanate of 17° Bé. per liter, squeezed out, predried at 60° C. and heated to 120° C. for 10 minutes, soaped, rinsed and loosely dried.

*Example 2.*—The treatment is the same as in Example 1, but after the untwisting of the yarn past the zero point it is steamed in a loose state.

*Example 3.*—Copperammonium artificial silk of a size of 120 denier and not twisted is given 2500 twists per meter. Then the yarn spools are steamed for 40 minutes at 4 atmospheres pressure. After drying the yarn is untwisted to the zero point and in this condition is cut into staple fibers on a suitable cutting machine. After

twisting of the staple fibers the yarn is treated with formaldehyde as described in Example 1.

*Example 4.*—Delusted copperammonium artificial silk yarn of a size of 150 denier with a twist of 200 per meter is supertwisted to 2000 twists per meter. Thereupon the supertwisted yarn which has been placed on bobbins is steamed at 5 atmospheres pressure for 20 minutes. After drying the yarn is untwisted on the twisting machine past the zero point and brought to 80 twists per meter in the opposite direction. Thereafter the yarn is steamed in the form of hanks and afterwards impregnated with a solution of 90 cc. formaldehyde 40% and 3 g. ammoniumchloride per liter, squeezed out, dried at 60° C. and treated to 120° C. for 15 minutes and finished as in Example 1.

*Example 5.*—The impregnation bath of Example 4 is replaced by the following bath:

Formaldehyde 40%-----cc. 100  
Technical zinc chloride per liter-----g. 20

the pH of the impregnation bath being brought if necessary to 4. The yarn is impregnated, squeezed out, dried at 60° C. and heated to 120° C. for 20 minutes and finished as in Example 1.

*Example 6.*—Viscose yarn of a size of 450 denier is supertwisted to 1250 turns per meter, steamed on bobbins at a pressure of 3 atmospheres for 40 minutes, dried and untwisted past the zero point and brought to 60 twists per meter in the opposite direction.

The so treated yarn is then woven into a pile fabric as pile yarn. After cutting the fabric is steamed without pressure for a sufficient time to produce the full curliness of the pile. Thereafter the fabric is impregnated on a padding machine with a solution containing per liter

Formaldehyde 40%-----cc. 100  
Aluminium thiocyanate solution  
of 17° Bé-----cc. 40

The excess liquid is squeezed off, the fabric dried on a stenter frame at 60° to 70° C. and then heated to 120° C. for 17 minutes preferably in a loop dryer. Thereafter the fabric is washed, soaped and finished in the usual way.

The fibrous material treated according to the above mentioned examples possesses a lasting curliness which resists repeated laundering and has great softness, the fibers being readily elongatable when subjected to a stretching force and being sufficiently elastic to return to or nearly to their original position upon discontinuance of said stretching force and contains a small amount of chemically bound formaldehyde.

I use the term "supertwist" or "supertwisting" herein with the same meaning as set forth in the specification of said prior U. S. Patent 2,019,185, commencing in line 47, first column, page 1 thereof, and ending in line 21, second column.

While the invention has been described in detail according to the preferred manner of carrying out the same, it will be obvious for those skilled in the art that changes and modifications may be made therein without departing from the spirit or scope of the invention.

What is claimed as new and desired to be secured by Letters Patent is:

1. A process for producing a new artificial fibrous material which comprises supertwisting an artificial silk yarn, setting the twist therein and thereafter untwisting the yarn to produce a wool-like effect, and combining this process with a treatment with formaldehyde or formaldehyde

yielding substances in the presence of acid reacting catalysts at temperatures of preferably 90-160° C.

2. Process for producing a new artificial fibrous material which comprises supertwisting an artificial silk yarn, setting the twist therein and thereafter untwisting the yarn to produce a wool effect, and combining this process with a treatment of the said material with formaldehyde or a formaldehyde-yielding substance, which treatment is as follows: impregnating the material with the formaldehyde or a formaldehyde-yielding substance in the presence of an acid catalyst having a dissociation constant above  $3 \times 10^{-4}$ , or a substance yielding such an acid at elevated temperature, removing the excess liquid and subjecting the said material to a temperature of above about 90° C. for a sufficient length of time

to form a formaldehyde-cellulose compound giving greater durability to the wool-like effect.

3. Process for producing a new fibrous material which comprises treating artificial silk fibers to render them wool-like and combining this treatment with a treatment of the said fibers which is as follows: impregnating the material with formaldehyde or a formaldehyde-yielding substance in the presence of an acid catalyst having a dissociation constant above  $3 \times 10^{-4}$ , or a substance yielding such an acid at elevated temperature, removing the excess liquid and subjecting the said material to a temperature above about 90° C. for a sufficient length of time to form a formaldehyde-cellulose compound giving greater durability to the wool-like effect.

GEORG HEBERLEIN.